

# UNITED STATES PATENT OFFICE.

FRANK MCPHILLIPS, OF TOLEDO, OHIO.

## WATERPROOFING COMPOSITION.

1,358,226.

Specification of Letters Patent. Patented Nov. 9, 1920.

No Drawing.

Application filed February 9, 1920. Serial No. 357,302.

To all whom it may concern:

Be it known that I, FRANK MCPHILLIPS, a citizen of the United States, residing at Toledo, county of Lucas, State of Ohio, 5 have invented a certain new and useful Improvement in Waterproofing Composition, and declare the following to be a full, clear, and exact description of the same, such as will enable others skilled in the art to which 10 it pertains to make and use the same.

My invention relates to a composition of matter for waterproofing and an object of my invention is to provide a waterproofing composition particularly adapted for use on 15 fabric materials such as automobile tops, tenting, tarpaulin, fish nets, et cetera.

A further object of my invention is to produce a waterproofing which will act as a preservative and not deleteriously affect 20 the fabric or material on which it is used, but which will increase the tensile strength of the fabric to which it is applied and will resist the action of salt water and acid fumes.

25 A still further object is to provide such a waterproofing material as may be used on metal parts such as anchor chains, bridge members and other metal pieces, or upon wood, such as boat hulls and decks. It will not injure the metal but will protect the 30 material from the action of the weather, salt water, or acid fumes.

My composition consists of a mixture of distillate of petroleum or other mineral oil, 35 gilsonite and fish oil, in substantially the following proportions:

Petroleum distillate 6 parts  
Gilsonite 3 parts  
Fish oil 1 part

40 The best results are secured, however, from a mixture in proportions approximately as follows:

Petroleum distillate 58.8%  
Gilsonite 35 %  
Fish oil 6.2%

A black pigment, preferably in the form of lamp black may be added which will

give the material coated a lustrous black 50 finish. This pigment should be added in the proportion of approximately .07% to  $\frac{1}{10}$ th of 1% and the preferred formula with the addition of lamp black would be as follows:

|                      |       |
|----------------------|-------|
| Petroleum distillate | 58.8% |
| Gilsonite            | 35 %  |
| Fish oil             | 6.1%  |
| Lamp black           | .1%   |

60

Each of these ingredients may vary widely in quality: Petroleum distillate particularly will be found to be of widely variable quality. In this connection, it has been found that the distillate resulting in 65 the refining of petroleum from the Texas and California oils best serves my purpose. Therefore, I do not wish to be understood as confining myself to the definite proportion hereinabove set forth. The distillate 70 or mineral oil used might vary from 50% to 70%, gilsonite from 20% to 40% and fish oil from 4% to 10% of the mixture.

The black pigment, if used, would be of small quantity, for although it possesses 75 waterproofing qualities, its principal purpose is as a coloring and for producing a finish.

The ingredients composing this compound would be thoroughly mixed, preferably at a temperature of from 50 to 70 degrees C. This mixture would preferably be applied to a fabric material such as tenting, or automobile tops, by being spread thereon with a brush. Fish nets and metal parts 80 might be immersed in a vat of the liquid. The best results would be secured at a temperature somewhat above 50 degrees C. 85

The number of coats or applications would depend on the character of the work 90 for which the material was intended and the weave of the fabric. If the composition were applied to a loosely woven, open-mesh fabric, more applications would be required to build up a waterproof coat. On the other hand, a closely woven fabric would require less.

Pantasote, used for automobile tops, pos-

seses a finished surface and close weave, when coated with the composition and dries with a lustrous black finish.

The composition dries better out of doors. 6 Good results are not obtained under the influence of artificial heat, unless there is a distinct air circulation.

This composition has been found to increase the tensile strength of cotton cloth 10 and burlap approximately one hundred per cent. Fabrics so treated resist the action of weather and salt water and are found to resist the action of acid fumes for days at a time. The pliable quality of the fabric 15 is in no way damaged; the coating will not crack or break and fabric so treated may be rolled or twisted without injury to the waterproofing applied thereto.

Metal parts may preferably be coated 20 with this composition by being immersed therein and will be found to be resistant to acid fumes thereafter, as well as the action of the weather and salt water. Metal is in no way corroded by the action of the composition.

This composition when used on hulls or decks of boats or other wooden material, might well contain distillate in as low a proportion as 20% to 50%, with a corre-

sponding higher percentage of gilsonite, 30 with practically no variation in the fish oil as above set forth.

I claim:

1. The within-described waterproofing composition, consisting of substantially six 35 parts of petroleum distillate, three parts of gilsonite, and one part of fish oil.

2. The within-described waterproofing composition, composed of mineral oil, gilsonite, fish oil, substantially as set forth. 40

3. The within-described waterproofing composition, consisting of petroleum distillate, gilsonite and fish oil substantially in the proportions set forth in the specification hereof. 45

4. The within described waterproofing composition consisting of about 59% petroleum distillate, about 35% gilsonite, about 6% fish oil, and a small quantity of lamp black. 50

5. The within-described waterproofing composition, composed of petroleum distillate 58.8 per cent., gilsonite 35 per cent., fish oil 6.1 per cent. and lamp black .1 per cent., substantially as described.

In testimony whereof I sign this specification.

FRANK McPHILLIPS.